

Nov. 12, 1935.

G. HEYMER

2,020,607

PHOTOGRAPHIC MATERIAL

Filed Dec. 5, 1931

Fig. 1



Fig. 2



Inventor:  
Gerd Heymer,  
By Attorney  
Philip S. Hopkins.

Patented Nov. 12, 1935

2,020,607

# UNITED STATES PATENT OFFICE

2,020,607

## PHOTOGRAPHIC MATERIAL

Gerd Heymer, Dessau-Ziebigk/Anhalt, Germany,  
assignor to Agfa Ansco Corporation, Bingham-  
ton, N. Y., a corporation of New York

Application December 5, 1931, Serial No. 579,350  
In Germany December 6, 1930

4 Claims. (CL 95—2)

My present invention relates to photographic materials for color-photography or stereo-photography.

One of its objects is to provide a process of manufacturing highly valuable color photographs which comprises equalizing the gradations of photographic layers arranged in succession and dyed each to have a different color, the dye being a constituent of the finished picture. 5 Another object is the photographic material provided with layers of similar gradation arranged in superposition and dyed each to have a different color, the dyes forming constituents of the finished pictures. Reference is made to the accompanying drawing which illustrates two films according to this invention.

In color-photography and stereo-photography there are required for some purposes photographic materials which contain the dye, necessary for the preparation of colored part pictures, in the emulsion layer already before the exposure to light. When using those materials it is sometimes difficult to obtain a tintless grey scale, because the curves of gradation of the single colored emulsion layers have not the same course. 25 This is particularly due to the coloration of the emulsion layer which acts in such a manner that, for instance, the greenish-blue coloration of an ordinary emulsion layer permeable to blue rays alters the original gradation only to a relatively small extent, whereas an orange-yellow coloration which is impermeable to blue rays, similarly to the known Dup-film, gives the colored emulsion a much flatter gradation.

According to my present invention this difficulty is avoided by assimilating the gradation of the photographic layers used together and dyed each to have a different color by incorporating in at least one of these layers a filter dye which absorbs at least part of the spectral region to which the layer in question is permeable and sensitive. The concentration of the filter dyes is regulated so that the gradations of the layers are equalized.

15 The colorations due to the filter dyes are after exposure removed in a bath in which the photographic material is to be treated, for instance, in the developing bath, fixing bath or another subsequent bath.

For equalizing, for example, red layers to green layers of a flatter gradation, for instance, methyl blue may be used. The coloration produced by this dye is easily removed in an aqueous solution of sodium sulfite. For changing the gradation 10 of a blue layer, for instance, tartrazine is well

appropriated, which is removable by washing with water. Green layers may be for altering the gradation additionally dyed with acid fuchsin, the coloration produced being removable by an aqueous solution of sodium sulfite. The 5 said removal of the filter dyes usually begins in the usual developing bath and is complete in the acid fixing bath.

The following example will most clearly illustrate my invention without limiting it: 10

On each face of a support a light sensitive emulsion layer is provided, one of which is dyed with Diamine green HS (see Schultz, Farbstofftabellen 1923, vol. II page 38) and the other is dyed with Salicinorange 2 R, a dye made from 15 nitrobenzidine, salicylic acid and 2-hydroxy-naphthalene-8-sulfonic acid, and with Benzo light red 8 B L (see Schultz, Farbstofftabellen 1923, vol. II page 19). The red dyed emulsion which is sensitized for red is furthermore treated with methylblue which equalizes the gradation of the red layer to that of the green layer which is sensitized for green. The proportion of the dyes used for the said layer may be about the following:

|                       | Parts by weight |
|-----------------------|-----------------|
| Salicinorange 2 R     | 80              |
| Benzo light red 8 B L | 4               |
| Methylblue            | 0.5             |

The concentration of the dyes in the single layers is chosen in such a manner that the red layer and the green layer give together a suitable black. The gamma value of the green layer is about 0.9 and that of the red layer without addition of methyl blue 1.5 to 2. After the addition of methyl blue the gamma value of the red layer likewise is about 0.9.

In order to manufacture a three-color film I may proceed, for instance, as follows:

The first emulsion layer is colored blue green by Brilliant benzo fast green. The second emulsion layer is colored purple by Sirius red violet R (cf. Chemisches Centralblatt 1928, vol. 1, page. 2461) or Sirius rubine B (cf. Chemisches Centralblatt 1931, vol. 2, page 364). The third emulsion layer is colored yellow by Benzo light yellow RL (cf. Fierz-David "Künstliche organische Farbstoffe" 1926, page 168) or Chrysophenine G extra (cf. Schultz, Farbstofftabellen 1931/JDC/ 45 726). In all these three layers the sensitiveness to red, green and blue light may be altered respectively by methyl blue, acid fuchsin and tartrazine.

In the annexed drawing, Fig. 1 shows a section 55

through the support *a* provided on one of its faces with a light sensitive emulsion layer *b* and on the opposite face with an emulsion layer *c*. The layer *b* comprises an emulsion layer, dyed green.

5 The layer *c* comprises an emulsion layer dyed red, sensitized for red and containing a blue-green filter dye for equalizing the gradation of this layer *c* to that of the layer *b*.

Fig. 2 shows a section through a support *a*, being provided on one of its faces with two light sensitive emulsion layers *b* and *c* and on the opposite face with a light sensitive emulsion layer *d*. The layer *c* comprises an emulsion layer dyed yellow sensitized for green and containing a red 10 filter dye. The layer *b* comprises an emulsion layer dyed purple sensitized for red and containing a blue-green filter dye. The layer *d* comprises a blue sensitive emulsion layer dyed blue-green and containing a yellow filter dye. The 15 amount of filter dye incorporated in each emulsion layer, is thus selected that the gradations of these layers are equalized. However, the addition of filter dye to one of the emulsion layers can be dispensed with if the gradations of the remaining 20 two layers are equalized to the gradation of the emulsion layer having the flattest gradation.

The quantity of the dye which is necessary for the equalization of the gradations depends upon the gradation and the sensitization of the emulsion used, upon the thickness of the layer and upon the kind of development. I do not wish to limit my invention to the foregoing examples nor to the specific details given therein. Numerous other embodiments are possible and I contemplate as included within my invention all such 30 modifications and equivalents as fall within the scope of the appended claims. Numerous other filter dyes for the purpose in question and known to every chemist skilled in the art may be employed. A few comparative experiments should be made to determine the most suitable filter dye and its most suitable amount to be used with a 35 particularly dyed emulsion for equalizing its gradation to that of a differently dyed emulsion.

40 45 What I claim is:

1. A photographic material comprising a sup-

port, on one face of said support a light-sensitive emulsion layer sensitized for green and dyed with Diamin Green HS and on the other face a light-sensitive emulsion layer sensitized for red and dyed with a mixture of Salycin Orange RR and Benzo light red 8 BL, the red dyed emulsion containing furthermore a substantial amount of 5 Methyl Blue for equalizing the gradation of the red layer to that of the green layer.

2. A photographic material comprising a support and at least two superimposed emulsion layers dyed to have different colors and colored for the same color to which the respective layer is specially sensitive, at least one of these emulsion layers containing furthermore a filter dye, soluble 10 in the photographic treating baths, which absorbs at least part of the spectral region which is transmitted by the color of this layer and to which this layer is sensitive, for equalizing the gradation of the emulsion layers. 20

3. A photographic material comprising a support and at least two superimposed emulsion layers in superposition being dyed to have different colors and colored for the same color to which the respective layer is specially sensitive, at least one of 25 these emulsion layers containing furthermore a filter dye, soluble in the photographic treating baths, which absorbs at least part of the spectral region which is transmitted by the color of this layer and to which this layer is sensitive, for 30 equalizing the gradation of the emulsion layers.

4. A photographic material comprising a support and at least two superimposed emulsion layers arranged on both faces of the support, said emulsion layers being dyed to have different colors 35 and colored for the same color to which the respective layer is specially sensitive, at least one of these emulsion layers containing furthermore a filter dye, soluble in the photographic treating baths, which absorbs at least part of the special 40 region which is transmitted by the color of this layer and to which this layer is sensitive, for equalizing the gradation of the emulsion layers.

GERD HEYMER. 45